

(No Model.)

C. C. GILMAN.

SIDEWALK.

No. 340,569.

Patented Apr. 27, 1886.



Attest:

Gov. H. Graham  
J. A. Healey

Inventor:

Chas. C. Gilman,  
per H. M. O'Brien,  
atty.

# UNITED STATES PATENT OFFICE.

CHARLES CARROLL GILMAN, OF ELDORA, IOWA.

## SIDEWALK.

SPECIFICATION forming part of Letters Patent No. 340,569, dated April 27, 1886.

Application filed October 15, 1885. Serial No. 179,917. (No model.)

*To all whom it may concern:*

Be it known that I, CHARLES CARROLL GILMAN, a citizen of the United States, and a resident of Eldora, Hardin county, Iowa, have 5 invented a new and useful Improvement in Sidewalks, of which the following is a specification.

The object of my invention is to construct a cheap and durable sidewalk having an indestructible and water-proof foundation which cannot be washed away by the action of water; and to this end my invention consists in using as a foundation for a surface layer of asphalt mastic or cement, blocks or slabs of 10 terra-cotta lumber or porous terra-cotta saturated or impregnated with asphaltum.

The accompanying drawing represents a cross-section of a sidewalk constructed in accordance with my invention.

20 The foundation of my sidewalk consists of blocks, A A', of terra-cotta lumber or porous terra-cotta, preferably three inches in thickness, about twelve inches wide, and from sixteen to thirty inches long. Said blocks are 25 saturated or impregnated with asphaltum. In order to thoroughly impregnate the slabs of said material with the asphaltum, I place the former in a closed tube, vessel, or receiver, from which I exhaust the air, and then admit 30 thereto the hot melted asphaltum, the same being forced by the atmospheric pressure into the pores or cells (exhausted of air) of the terra-cotta lumber, the latter being heated to about the same or greater temperature as the 35 said asphaltum, to avoid chilling the latter.

The method just described is similar to the well-known process employed in impregnating wood with creosote, and since no claim is laid to said method, a fuller description there- 40 of is not essential to an understanding of this invention.

The saturated terra-cotta lumber, after it has cooled and the asphaltum hardened or become solid, is in fact a new material, which is 45 much stronger and of greater weight than the unimpregnated material, is absolutely imper- vious to moisture, cannot decay, and is prac- tically indestructible.

The said slabs or blocks, treated as de-

scribed, are arranged in two layers, so as to 50 break joints with each other in both directions. The lower blocks, A', rest preferably on a foundation of sand or gravel, B. These two layers of indestructible and water-proof material make a solid foundation for the surface covering. The upper blocks, A, are cov- 55 ered with a layer of asphalt mastic, C, composed of asphalt, gravel, and pounded lime- stone. This mastic is rolled over the same to a thickness of from one to two inches, varying 60 according to circumstances.

I do not wish to limit myself to a formation consisting of two layers of blocks, as one layer of thicker blocks may be used, or the blocks may be formed so as to have a bearing on each 65 other; but the construction illustrated is much to be preferred. Neither do I desire to limit myself to a wearing-surface of asphalt mastic, for a layer of cement may be used in lieu thereof. It is evident, also, that my inven- 70 tion is applicable to street-pavements as well as to sidewalks; but in the construction of pavements a stronger foundation and a thicker layer of asphalt mastic is used.

I am aware that ordinary building-bricks 75 have been immersed in a liquid solution of alum, borax, copperas, and water, and after drying boiled in a mixture of caoutchouc and coal-tar, and that it has been proposed to use such bricks as the surface layer of a pavement 80 or sidewalk. I am also aware that it has been proposed to lay a surface layer of terra-cotta blocks upon a foundation of bricks, and also that it is not new to cure a brick by immerge- 85 gion in a mixture of coal-tar, bitumen, pine- gum, and alum; and these several things I do not claim.

I am aware that a roller-skating surface has been formed by laying on a foundation of ordinary brick a composition of asphalt, bitu- 90 men, and resinous oil; but this I do not claim, as it is entirely different from my invention.

Having thus described my invention, what I claim, and desire to secure by Letters Patent, is—

1. A sidewalk or pavement consisting of a surface layer of asphalt mastic or its equivalent and a foundation composed of slabs or

blocks of terra-cotta lumber saturated or impregnated with asphaltum, substantially as described.

2. A sidewalk or pavement consisting of a 5 surface layer of asphalt mastic or its equivalent and a foundation composed of two layers of blocks of terra-cotta lumber saturated or impregnated with asphaltum and arranged to

break joints with each other in both directions, substantially as described.

In testimony whereof I have signed my name in the presence of two witnesses.

CHARLES CARROLL GILMAN.

Witnesses:

SAML. G. SLOAN,  
H. H. GALUSHA.